

# United States Patent Office

2,931,737

Patented Apr. 5, 1960

1

2,931,737

## IMPREGNATION PROCESS

**Jesse Thornton, Leeds, England, assignor to Hickson's  
Timber Impregnation Co. (G.B.) Limited, Castleford,  
England, a British company**

No Drawing. Application April 4, 1958  
Serial No. 726,316

Serial No. 7,26,516  
**Claims priority, application Great Britain July 30, 1957**  
**4 Claims (Cl. 117 - 116)**

This invention is concerned with improvements in or relating to impregnation processes, and is more particularly concerned with the impregnation of fibreboard materials with liquids, such as aqueous solutions containing, for example, fire-retardants and/or preservatives, and/or with aqueous solutions of resins capable of imparting dimensional stability.

By the term "fibre-board" as used herein we means any board which has been manufactured by compression of comminuted cellulose, such as insulation board and wall board and also includes such materials as cardboard which are made under light compression as well as the more solid type of board. The term does not, however, include fibre-boards which are of such a solid nature that it is not feasible to impregnate them, for example such boards as have a hardness comparable to that of metal or such as have a density in excess of  $720 \text{ kg./m}^3$ .

Untreated fibre-board suffers from the disadvantage that it is combustible to a varying degree and various attempts have been made to impart a fire-retardancy to such board by impregnating it with fire-retarding solutions. The methods so far proposed, however, have not been commercially successful. Thus, one method which has been tried is to incorporate the fire-retardant compounds into the slurry which is used in the manufacture of the fibre-board, but this has been found to be commercially impracticable as it interferes with the manufacturing process; furthermore the amount of impregnant which is incorporated in the fibre-board cannot be controlled accurately and, in addition, there is considerable waste of impregnant.

It is also virtually impossible to impregnate fibre-board by merely immersing the manufactured board in an impregnant solution as the board becomes virtually impossible to handle in the wet state because it becomes soft.

Various processes are now well-known for impregnation of timber with, for example, preservative solutions and examples of such processes include various pressure/vacuum impregnation processes. Timber, however, has a continuous cellular structure and consists substantially of a mass of inter-connected cells. Fibre-boards with which the present invention is concerned have, however, a discontinuous structure and thus the problem of their impregnation should differ radically from the impregnation of timber. We have, however, found that one of the impregnation processes developed for treating timber (and dependent on the continuous cellular structure thereof), namely the Rueping process, is capable of adaptation to the successful impregnation of fibre-board despite the discontinuous structure of the latter.

The Rueping process for the treatment of timber consists basically in forcing air or other gas under pressure into the timber to be impregnated and then forcing the impregnant liquid into the timber at a higher pressure than that at which the air or other gas was introduced. After a certain time the pressure is released and, if desired, a vacuum is applied to the timber when a large quantity of the impregnant is forced out of the timber by the gas contained therein under pressure. By controlling the initial gas pressure and the pressure at which the liquid is forced into the timber, and, if desired, the time

of impregnation, the amount of impregnant introduced into the timber can be controlled as well as the depth of impregnation.

According to the invention, therefore, we provide a process for the impregnation of fibre-board with an impregnant liquid in which the fibre-board is subjected in a pressure vessel to an initial gas, preferably air, pressure, impregnant liquid is then introduced into the pressure vessel under a pressure greater than that of the initial gas pressure to force the impregnant liquid into the fibre-board against the initial gas pressure to the desired degree of impregnation after which the liquid pressure is released.

15 A further measure of control of the amount of impregnation may be secured by variation of the time within which said liquid pressure is applied.

The process according to the invention is conveniently carried out for example using a conventional vacuum/pressure impregnation plant as used for the impregnation 20 of timber. Other methods of operation can of course be used.

By the process according to the invention it is possible to impregnate fibre-board to any desired degree and to achieve any desired depth of impregnation. This represents a considerable advance in the art as fibre-board is very absorbent and immersion in liquid for very short periods results in a very high volumetric absorption. Thus, if reference is made to the table set out below it will be seen that the absorption in litres per cubic metre of fibre-board of impregnant is very high even after only a few minutes immersion.

| Duration of Immersion |       | Absorp-tion in Litres/m. <sup>3</sup> |
|-----------------------|-------|---------------------------------------|
| Mins.                 | Secs. |                                       |
| 0                     | 15    | 333                                   |
| 0                     | 30    | 436                                   |
| 1                     | 0     | 502                                   |
| 2                     | 0     | 552                                   |
| 3                     | 0     | 663                                   |
| 4                     | 0     | 727                                   |
| 5                     | 0     | 776                                   |

45 From the above table it is apparent that it would not be possible to achieve accurate control of impregnation of fibre-board merely by immersing the fibre-board in a solution of an impregnant for a certain time and removing the fibre-board after such a time interval, as absorption of the impregnant is so rapid. By the process according to the invention, however, it is possible to achieve control of the impregnation process which has not hitherto been possible.

Thus if reference is made to the table set out below it will be seen that the absorption of impregnant in litres per cubic metre of fibre-board can be controlled to a very fine degree.

### TREATMENT CYCLE

From the above table it will be apparent that it is possible to control accurately the absorption of the impregnant within the range of about 65-500 litres/m.<sup>3</sup>, the latter quantity of impregnant being in general sufficient to impart substantially complete fire-retardancy to the fibre-board being treated whilst a quantity of about 65 litres/m.<sup>3</sup> would impart a considerable fire-retardancy to the surface of the fibre-board. It should be noted in this connection that it may often only be necessary to impart a fire-retardancy to the surface of fibre-board and that by the process according to the invention it is possible to control the depth of impregnation to a considerable degree. Thus, in Example 1 of the above table the fibre-board is impregnated to a depth of approximately 3.2 mm., leaving the centre core of the board dry and free from fibre-retardant.

The process according to the invention gives the best results when operated within certain pressure and time limits which are set out in the table below.

| Initial Air Pressure           |      |                    |      | Impregnant Pressure            |      |                    |      | Final Vacuum   |      |                    |      |
|--------------------------------|------|--------------------|------|--------------------------------|------|--------------------|------|----------------|------|--------------------|------|
| Pressure, Kg./cm. <sup>2</sup> |      | Time Held, minutes |      | Pressure, Kg./cm. <sup>2</sup> |      | Time Held, minutes |      | Vacuum, mm./Hg |      | Time Held, minutes |      |
| Min.                           | Max. | Min.               | Max. | Min.                           | Max. | Min.               | Max. | Min.           | Max. | Min.               | Max. |
| 1                              | 3    | 5                  | 20   | 1.5                            | 7    | 10                 | 60   | 254            | 735  | 5                  | 60   |

As will be seen from the above table, it is preferred that the initial air pressure be within the range of 1-3 kg./cm.<sup>2</sup> and that it should be maintained for 5-20 minutes. Preferably the pressure of the impregnant liquid introduced after the air has been introduced is within the range of 1.5-7 kg./cm.<sup>2</sup> and such pressure should first be maintained for 10-60 minutes. Finally, it is preferred that a vacuum of 250-740 mm./Hg be applied after the impregnant liquid has been introduced, such vacuum being maintained for a time within the range of from 5-60 minutes.

The process according to the invention can be used for the impregnation of fibre-board with any desired liquids. In practice, such liquids will often be aqueous solutions containing for example fire-retardant salts or preservative salts or aqueous solutions of resins capable of producing dimensional stability in the fibre-board. Where aqueous salt solutions are used the concentrations employed can vary as desired and in the case of fire-retardant compositions may, for example, contain from 50 5-30, preferably 10-20% of fire-retardant substances.

Any desired compound may be used in the impregnating solution according to the invention; such solutions may comprise fire-retardant or a mixture of fire-retardant compounds, for example, monoammonium dihydrogen phosphate, ammonium sulphate, borax and the like. Preservative compounds which may be used include disodium arsenate, sodium fluoride, sodium chromate, copper sulphate and the like.

In this connection, it should be noted that previously the Rueping process has not, as far as is known, been applied to impregnation of timber using aqueous solutions. This is because no advantage would normally be gained by using the Rueping process for the impregnation of timber using aqueous solutions as other methods of impregnation are equally applicable. It is only where it is desired to conserve the solvents containing the impregnant as much as possible that one applies the Rueping process because in this process a large quantity of the impregnant is forced out under pressure after impregnation has taken place. Thus, it is only in the case where recovery is important that the Rueping process has been applied.

In the process according to the invention, however, it is only by applying the Rueping process that one can

achieve control of the impregnation process. The process according to the invention is, of course, not restricted to the use of aqueous solutions but could equally well be applied to non-aqueous solutions. In practice it is very often preferable to impregnate with aqueous solutions thus avoiding use of expensive solvents so that the present invention particularly includes the use of aqueous impregnant solutions.

The process according to the invention can clearly be applied to the impregnation of fibre-board with any desired solution and is not restricted to imparting fire-retardancy thereto. Thus the solution used for impregnation may contain preservatives as well as or in place of fire-retardants; they may also contain resins for imparting dimensional stability. In fact, it may often be desirable to incorporate both fire-retardants and preservatives into the fibre-board being treated as well as resins for imparting dimensional stability.

After the fibre-board has been subjected to the im-

pregnation process it can be dried in any convenient manner.

It will be appreciated that by the process according to the invention it is possible to impregnate fibre-board for example to impart a fire-retardancy thereto and/or incorporate preservatives and/or resins therein in any desired amount, without substantial damage to the fibre-board.

In order that the invention may be well understood the following examples are given by way of illustration only:

#### Example 1

##### 1.27 CM. FIBRE INSULATION BOARD

###### Treatment cycle:

Initial air pressure..... 2.12 kg./cm.<sup>2</sup>, 10 mins.  
Solution pressure..... 3.18 kg./cm.<sup>2</sup>, 30 mins.  
Vacuum..... 625 mm. Hg., 15 mins.  
Absorption..... 190 litres/m.<sup>3</sup>  
Fire retardant solution..... Monoammonium dihydrogen phosphate, ammonium sulphate and borax.  
Solution strength..... 15%  
Net dry salt retention..... 40.0 kg./m.<sup>3</sup>.

#### Example 2

##### 1.89 CM. THICK FIBRE INSULATION BOARD TILES

###### Treatment cycle:

Initial air pressure..... 2.82 kg./cm.<sup>2</sup>, 10 mins.  
Solution pressure..... 4.23 kg./cm.<sup>2</sup>, 35 mins.  
Initial vacuum..... 609 mm. Hg., 12 mins.  
Absorption..... 330 litres/m.<sup>3</sup>  
Fire retardant solution..... Monoammonium dihydrogen phosphate, ammonium sulphate and borax.  
Solution strength..... 15%  
Net dry salt retention..... 48.0 kg./m.<sup>3</sup>.

#### Example 3

##### 1.27 CM. FIBRE INSULATION BOARD

###### Treatment cycle:

Initial air pressure..... 2.12 kg./cm.<sup>2</sup>, 10 mins.  
Solution pressure..... 2.82 kg./cm.<sup>2</sup>, 30 mins.  
Absorption..... 145 litres/m.<sup>3</sup>  
Solution..... Disodium arsenate, sodium fluoride, sodium chromate.  
Solution strength..... 4%  
Net dry salt retention..... 8.0 kg./m.<sup>3</sup>.

###### I claim:

1. A process for the controlled impregnation with an impregnant liquid of a highly absorbent fibre-board of compressed comminuted cellulose having a density not exceeding 720 kg./m.<sup>3</sup>, comprising subjecting the fibre-board in a pressure vessel to an initial superatmospheric

gas pressure not greater than 3 kg./cm.<sup>2</sup> for from 5-20 minutes, introducing impregnant liquid into the pressure vessel under a pressure greater than that of the initial gas pressure but not greater than 7 kg./cm.<sup>2</sup> for from 10-60 minutes to force the impregnant liquid into the fibre-board against the initial gas pressure to obtain a relatively high concentration of impregnant in the outer portions of said fibre-board while leaving the centre portion of said fibre-board substantially free of impregnant and releasing the liquid pressure.

2. A process as claimed in claim 1 in which a vacuum

of from 254-735 mm. Hg is applied to remove excess impregnant liquid after release of the liquid pressure.

3. A process as claimed in claim 2 in which the vacuum is applied for a period of from 5-60 minutes.

5. 4. A process as claimed in claim 1 in which said impregnant liquid is an aqueous solution.

References Cited in the file of this patent

UNITED STATES PATENTS

- 10 1,523,925 Wheaton ----- Jan. 20, 1925  
1,556,570 Coolidge ----- Oct. 6, 1925